

## UNITED STATES PATENT OFFICE

KARL HUERTTLE, OF AKRON, OHIO, ASSIGNOR TO GOODYEAR-ZEPPELIN CORPORATION,  
OF AKRON, OHIO, A CORPORATION OF DELAWARE

## GAS CONTAINER FOR AIRCRAFT

No Drawing.

Application filed January 27, 1928. Serial No. 250,071.

My invention relates to gas containers for lighter-than-aircraft and it has particular relation to methods of treating fabric for such containers whereby to render them impermeable to inflating gases.

More specifically the invention has for one of its objects the provision of a material for coating gas cell fabric which is highly impermeable to gases, relatively inexpensive to manufacture, and which is extremely durable.

It is customary in the construction of the gas containers for lighter-than-aircraft to apply an impermeable film to the surface 15 of the fabric in order to prevent diffusion of the gas. Heretofore, the most satisfactory material for this purpose has been gold beater's skin, a thin membrane taken from the intestines of animals. However, this 20 material is relatively expensive and it is also obtained in the form of small sheets which must be trimmed and which require a great amount of labor to apply, when extensive surfaces are to be coated therewith.

Rubber cements have, also, been employed 25 as gas proofing media. These cements are comparatively inexpensive and may be readily applied to the fabric by mechanical means such as ordinary calender rolls.

However, coating films formed of rubber have a much higher degree of permeability 30 than gold beater's skin and are, therefore, objectionable due to the relatively high loss of inflating gas by diffusion.

Numerous substitutes for gold beater's skin and for rubber films have, heretofore, been suggested. Among the materials proposed are gelatin and various cellulose derivatives such as nitrocellulose, cellulose 35 acetate and other compounds of this class. Coatings formed of these materials have proved unsatisfactory for various reasons, some of them being unduly permeable to the inflating gas while others are stiff and do 40 not adhere readily to the fabrics. They, therefore, quickly crack and peel from the fabric when placed in service.

This invention consists in the discovery 45 that fabrics coated with solutions or varnishes of phenyl resin, more commonly

known as "bakelite", when suitably treated and applied to gas cells, produce coating films which are highly resistant to the diffusion of gases, durable, flexible and which may be obtained and applied to the fabrics 55 at small expense.

In the practice of this invention, a bakelite varnish is mixed with a suitable softener such as castor oil, tricresyl phosphate, triphenyl phosphate, or other suitable softening agent. If desired, it may also be mixed 60 with a thinning agent such as acetone. It is then applied to a fabric by means of a spray, or by painting, or by calendering it upon fabric. The latter should be light in 65 weight, but of a strong closely woven texture. Special grades of cotton fabric are usually employed for this purpose, although silk and linen may be employed in certain cases.

The coated fabric is stretched and dried 70 while it is heated, preferably by training it about slowly moving rollers within a drying oven. The temperature of this oven should be maintained at 90° to 100° C., although these limits may under certain circumstances be varied. The fabric should remain in the drying oven for a period of 75 from one to two hours.

The proportions of the various ingredients 80 may vary within relatively wide limits, but the following are examples of formulæ which are found to give excellent results:

(1) 100 grams of bakelite varnish, 15 grams of castor oil and 225 cc. of acetone. 85  
(2) 50 grams of varnish, 10 grams of tricresyl phosphate and 200 cc. of acetone.  
(3) 50 grams of bakelite varnish, 5 grams of tricresyl phosphate, 10 grams of castor oil and 200 cc. of acetone.

(4) 50 grams of bakelite varnish, 15 grams of tricresyl phosphate and 200 cc. of acetone.

The bakelite varnish employed in these formulæ was of the grade known as "No. 1 95 clear", prepared by the Bakelite Company, Perth Amboy, N. J. It is to be understood that any good grade of bakelite varnish or lacquer may be used.

As previously stated, the castor oil and 10

tricresyl phosphate are added to the bakelite varnish, in order to render the finished product tough and flexible. The acetone is added for the purpose of thinning the varnish, in order that it may be spread thinly and evenly upon the fabric. The proportions of the thinning agent may of course be varied at will. If it is desired to coat the fabric with a single film, the proportion of acetone should be relatively small so that a comparatively thick coating may be applied at a single application. If it is desired that the coating should consist of a plurality of thin films of varnish, the latter should be first thinned with a relatively large quantity of acetone, in order that it may be spread with sufficient thinness upon the fabric to permit the application of a relatively large number of coats without rendering the product unduly heavy.

The application of a plurality of thin coats is, in many respects, preferable to the application of a single thick coating, because during the evaporation of the bakelite solvent, small bubbles may escape leaving pores and openings in the coating. If a number of films are applied, each preceding coating being dried before the application of the second coating, the probability of a number of interstices or openings coming into alignment with each other is relatively slight. Although acetone has been specified as a thinning agent, other suitable bakelite solvents are the equivalent thereof and the invention is, therefore, not limited to that particular compound.

After the fabric has been coated and dried it is cut into pieces of suitable shape and the pieces are then fastened together by cement or other convenient means in order to form gas containers of the desired shape and size.

Although I have described in detail only the preferred embodiments of the invention, it will be apparent to those skilled in the art that it is not so limited, but that various minor modifications may be made therein without departing from the spirit of the invention or from the scope of the appended claims.

What I claim is:

1. A gas cell for lighter-than-aircraft comprising a fabric coated with bakelite.
2. A gas cell for lighter-than-aircraft comprising a fabric coated with bakelite containing a softening agent.
3. A gas cell for lighter-than-aircraft comprising a closely woven fabric coated with bakelite containing tricresyl phosphate.
4. A gas cell for lighter-than-aircraft comprising a fabric coated with a material comprising bakelite, tricresyl phosphate and castor oil.
5. A gas cell for lighter-than-aircraft

comprising a fabric coated with bakelite containing castor oil.

In witness whereof, I have hereunto signed my name.

Signed at Akron, in the county of Summit and State of Ohio, U. S. A., this 26th day of January, 1928.

KARL HUERTTLE.